

# United States Patent Office

**2,972,571**

Patented Feb. 21, 1961

1

2,972,571

## NICKEL PLATING SOLUTIONS

Jack L. Towle, Cleveland, Ohio, assignor to The Harshaw Chemical Company, Cleveland, Ohio, a corporation of Ohio

No Drawing. Filed Feb. 10, 1960, Ser. No. 7,784

7 Claims. (Cl. 204—49)

This invention, which is a continuation-in-part of co-pending application Serial No. 833,398, filed August 13, 1959, now abandoned, relates to electrodeposition of bright nickel, that is to the production of bright deposits of nickel which are bright as taken from the electroplating solution without buffing or polishing of any kind, and to the composition of solutions suitable for the production of such deposits.

Various solutions are known which are capable of producing bright nickel deposits. Some of these are of commercial value. Some are superior in particular respects while being inferior in other respects. Brightness, resistance to corrosion, long periods of trouble-free operation, adherence, ductility, freedom from pits, streaks and other irregularities, resistance to impurities in the bath are some of the factors which the art seeks to find in high degree and as many as possible in one process.

I have now discovered a group of closely related classes of compounds which are excellent additives for use in acid nickel plating when used in connection with the aromatic sulfonates, sulfonamides and sulfimides. The latter may be referred to as control agents, the former as brighteners or auxiliary brighteners.

The class of brighteners with which the concerned are those having the formula



wherein R is a member selected from the group consisting of  $-\text{H}$ ,  $-\text{CN}$ ,

**2**

$$-\overset{\text{S}}{\text{C}}(\text{CH}_2)_n\text{CN},$$


$$\text{CH}_3(\text{CH}_2)_n'\text{S}-$$


W is a hydrocarbon radical and preferably a hydrocarbon radical having from 1 to 7 carbon atoms; X is an acid radical selected from the group consisting of sulfate, sulfonate, halide and perchlorate radicals; n is an integer from 1 to 6, and n' is an integer from 1 to 6.

The classes of brighteners referred to are as follows:

$$10 \quad (1) \quad \begin{array}{c} S[(CH_2)_nCN]_2 \\ | \\ W-X \end{array}$$

where W is a hydrocarbon radical, X is an acidic radical selected from the group consisting of

15                     $-\text{OSO}_2\text{OR}$  and  $-\text{OSO}_2$   R

where R is a hydrocarbon radical and n is an integer from 1 to 2 inclusive.

$$20^{(2)} \quad \begin{array}{c} R(CH_2)_nS(CH_2)_n \\ | \\ W \quad X \end{array}$$

where R is an alkyl group, W is a hydrocarbon radical, XX is an acidic radical selected from the group consisting of  $-\text{OSO}_2\text{OR}'$ , where R' is a hydrocarbon radical

25 

where  $R'$  is a hydrocarbon radical and  $n$  is an integer from 1 to 2 inclusive.

30 (3)  $\text{NC}(\text{CH}_2)_n\text{S}(\text{CH}_2)_n\text{S}(\text{CH}_2)_n\text{CN}$

where W is a hydrocarbon radical, X is an acidic radical selected from the group consisting of  $-\text{OSO}_2\text{OR}$

$$\text{O}_2\text{S}(\text{O})_2\text{R}$$

where R is a hydrocarbon radical,

Specific examples of brightener compositions according

Specific examples of eight applications of the invention to the invention are set forth in Table I below:

Table 1.

| No. | Structure                                                                                                                                                                                                                                                                                                                                                                              | Name                                                          | Preferred Concentration, Grams per Liter |
|-----|----------------------------------------------------------------------------------------------------------------------------------------------------------------------------------------------------------------------------------------------------------------------------------------------------------------------------------------------------------------------------------------|---------------------------------------------------------------|------------------------------------------|
| 1   | $\text{NC}-\text{CH}_2-\text{CH}_2-\overset{+}{\text{S}}-\text{CH}_2-\text{CH}_2-\text{CN}$ <div style="text-align: center; margin-left: 100px;"> <math>\text{C}_2\text{H}_5</math>      <math>\text{OSO}_2\text{OC}_2\text{H}_5</math> </div>                                                                                                                                         | Ethyl bis (B-cyanoethyl) sulfonium ethyl sulfate.             | .003-.02                                 |
| 2   | $\text{NC}-\text{CH}_2-\text{CH}_2-\overset{+}{\text{S}}-\text{CH}_2\text{CH}_2\text{CN}$ <div style="text-align: center; margin-left: 100px;"> <math>\phi\text{CH}_2</math>      <math>\text{I}^-</math> </div>                                                                                                                                                                       | Benzyl bis (B-cyanoethyl) sulfonium iodide.                   | .003-.02                                 |
| 3   | $\text{NC}-\text{CH}_2\text{CH}_2-\overset{+}{\text{S}}-\text{CH}_2\text{CH}_2-\text{S}-\text{CH}_2\text{CH}_2\text{CN}$ <div style="text-align: center; margin-left: 100px;"> <math>\text{C}_2\text{H}_5</math>      <math>\text{O}-\text{SO}_2\text{OC}_2\text{H}_5</math>      <math>\text{C}_2\text{H}_5</math>      <math>\text{O}-\text{SO}_2\text{OC}_2\text{H}_5</math> </div> | 1,2-ethylene-bis (B-cyanoethyl ethyl sulfonium ethylsulfate). | .003-.02                                 |
| 4   | $\text{CH}_3\text{CH}_2\text{CH}_2-\overset{+}{\text{S}}-\text{CH}_2\text{CH}_2\text{CN}$ <div style="text-align: center; margin-left: 100px;"> <math>\text{C}_2\text{H}_5</math>      <math>\text{O}-\text{SO}_2\text{OC}_2\text{H}_5</math> </div>                                                                                                                                   | B-cyanoethyl propylethylsulfonium ethyl sulfate.              | .003-.02                                 |
| 5   | $\text{NC}-\text{CH}_2\text{CH}_2-\overset{+}{\text{S}}-\text{CH}_2\text{CH}_2\text{CN}$ <div style="text-align: center; margin-left: 100px;"> <math>\text{CH}_3</math>      <math>\text{O}-\text{SO}_2</math>  <math>\text{CH}_3</math> </div>                                                     | Methyl-bis (B-cyanoethyl) sulfonium p-toluene sulfonate.      | .003-.02                                 |
| 6   | $\text{CH}_3\text{CH}_2\text{CH}_2-\overset{+}{\text{S}}-\text{CH}_2\text{CH}_2\text{CN}$ <div style="text-align: center; margin-left: 100px;"> <math>\text{C}_2\text{H}_5</math>      <math>\text{OS-O}_2</math>  <math>\text{CH}_3</math> </div>                                                  | Ethylpropyl-B-cyanoethyl sulfonium p-toluene sulfonate.       | .003-.02                                 |

The second addition agent, which cooperates with the brightener in bright, acid, nickel plating solutions falls into the category of organic sulfonamides, sulfimides, and sulfonates.

The amount of control agent dissolved in the acid nickel plating solution ranges from .05 gram per liter to 20 grams per liter, best results being obtained from about 2 to about 5 grams per liter. These may be used in admixture as well as singly. That is, two control agents 10 may be used instead of one, their combined concentration being kept within the above indicated limits.

Table II  
AROMATIC SULFONAMIDES

|                                                        |                                                    |
|--------------------------------------------------------|----------------------------------------------------|
| benzene monosulfonamide                                | $C_6H_5SO_2NH_2$                                   |
| saccharine, sodium salt                                | $C_6H_5SO_2CONa$                                   |
| $\rho$ -toluenesulfonamide                             | $CH_3C_6H_4SO_2NH_2$                               |
| trichlorodibenzene sulfonamide                         | $Cl_3C_6H_2SO_2NHSO_2C_6H_4Cl$                     |
| di- $\beta$ -naphthalenesulfonamide                    | $C_10H_7SO_2NHSO_2C_10H_7$                         |
| 4-carboxydibenzene sulfonamide                         | $C_6H_5SO_2NHSO_2C_6H_4COOH$                       |
| $N,N'$ -bis(phenylsulfonyl)-4,4'-diphenyldisulfonamide | $C_6H_5SO_2NHSO_2C_6H_4C_6H_5SO_2NHSO_2C_6H_4$     |
| $\rho,\rho'$ -oxy-bis(dibenzenesulfonamide)            | $C_6H_5SO_2NHSO_2C_6H_4O_2C_6H_5SO_2NHSO_2C_6H_4$  |
| $\rho,\rho'$ -methylene-bis-(dibenzenesulfonamide)     | $C_6H_5SO_2NHSO_2C_6H_4CH_2C_6H_4SO_2NHSO_2C_6H_4$ |

## AROMATIC SULFONATES

|                                 |                       |
|---------------------------------|-----------------------|
| benzene monosulfonic acid       | $C_6H_5SO_2H$         |
| benzene disulfonic acid         | $C_6H_4(SO_2H)_2$     |
| nickel naphthalene disulfonate  | $C_{10}H_8(SO_2)_2Ni$ |
| cobalt naphthalene disulfonate  | $(C_6H_5SO_2)_2Co$    |
| nickel benzene monosulfonate    | $(C_6H_5SO_2)_2Ni$    |
| dichlorobenzene disulfonic acid | $Cl_2C_6H_4(SO_2H)_2$ |
| toluene sulfonic acid           | $CH_3C_6H_4SO_3H$     |
| diphenyl sulfonic acid          | $C_6H_5C_6H_4SO_3H$   |
| thiophene sulfonic acid         | $C_4H_8S_2SO_3H$      |
| diphenyl sulfone                | $C_6H_5SO_2C_6H_5$    |
| naphthalene trisulfonic acid    | $C_{10}H_8(SO_2OH)_3$ |

## UNSATURATED ALIPHATIC SULFONAMIDES AND SULFONIC ACIDS

|                        |                       |
|------------------------|-----------------------|
| sodium vinyl sulfonate | $H_2C=CHSO_3Na$       |
| sodium allyl sulfonate | $H_2C=CHCH_2SO_3Na$   |
| vinyl sulfonamide      | $H_2C=CHSO_2NH_2$     |
| allyl sulfonamide      | $H_2C=CHCH_2SO_2NH_2$ |

The constituents of the plating bath, according to the preferred practice of the invention, are (1) water, (2) nickel sulfate, nickel chloride, or a mixture of nickel sulfate and nickel chloride, (3) the brightener, (4) a sulfonate, a sulfonamide, a sulfimide, or one or more sulfonates, sulfonamides, sulfimides or mixtures thereof of the type previously indicated, (5) and a wetting agent (optional). An additional ingredient of the solution which is desirable is a buffering agent such as boric acid, 55 formic acid, or the like.

It will be noted that in reference to the major constituent of the nickel plating solution, the solutions are similar to the well known "all chloride," "all sulfate," and "sulfate-chloride" or "Watts" type acid nickel plating solutions. The essential novel feature of the invention is the use of an acid nickel plating solution having one or more nickel electrolytes selected from nickel sulfate and nickel chloride and additionally containing cooperating brightening agents, one of which is at least one carrier selected from the group consisting of unsaturated aliphatic sulfonamides, unsaturated aliphatic sulfimides, unsaturated aliphatic sulfonates, aromatic sulfonamides, aromatic sulfimides and aromatic sulfonates, and the other of which is a small amount of a brightener of the type heretofore indicated. 70

The basic solutions in connection with which the bright ductile nickel deposits are realized when containing the cooperating addition agents dissolved therein are as follows:

## SULFATE-CHLORIDE WATTS TYPE

|                                            |                                                                         |
|--------------------------------------------|-------------------------------------------------------------------------|
| $NiSO_4 \cdot 7H_2O$                       | 100 to 400 grams, preferably 200 to 300 grams.                          |
| $NiCl_2 \cdot 6H_2O$                       | 10 to 60 grams, preferably 25 to 40 grams.                              |
| Boric acid                                 | 0 to 50 grams, preferably 15 to 40 grams.                               |
| Wetting agent (e.g. sodium lauryl sulfate) | 0 to 0.5 gram, preferably 0.025 to 0.2 gram.<br>$H_2O$ to make 1000 cc. |

The plating solutions above identified may be operated under conditions of pH, temperature, and cathode current density which are customarily employed therewith. When the cooperating brightening agents of the invention are dissolved in the plating solutions in the amount previously indicated, bright, ductile deposits will be obtained upon electrolysis of the solution. Typical operating conditions for the basic solutions are as follows:

|                                                  | All Sulfate | All Chloride | Watts   |
|--------------------------------------------------|-------------|--------------|---------|
| pH                                               | 3-4.5       | 2.4-4.5      | 3-4.5   |
| Temperature, °F.                                 | 120-160     | 100-150      | 110-155 |
| Cathode Current Density (amp./ft. <sup>2</sup> ) | 20-40       | 60-200       | 30-70   |

In the preparation of the plating solution according to the invention, I add to each of the foregoing basic solutions a suitable quantity of the brightener and also one or more of the unsaturated aliphatic, or aromatic sulfonamides, sulfimides, and sulfonates. The plating solu-

tion for the best results, contains an antipitting agent although the deposits may be suitable for some purposes without eliminating pitting. Sodium lauryl sulfate or other wetting agents, such as the sodium sulfate derivative of 7-ethyl-2-methylundecanol-4 and the dihexyl ester of sodium sulfosuccinic acid may be used as an antipitting agent, although its use is not essential and other wetting agents or mixtures of wetting agents may be used to control the pitting. For some purposes pitting may be tolerated and sometimes very little pitting occurs.

Specific examples of electroplating solutions containing different cooperating brighteners and carriers are illustrated in the following table designated as Table III. It should be understood that these specific electroplating solutions may be used with or without air agitation. The operating conditions for obtaining bright ductile nickel deposits are also set forth in the table. In each case a bright nickel deposit of from 0.05 to about 1 mil thick or thicker may be secured by electrolyzing the electroplating solution between an anode and a buffed brass cathode. Similar results may be secured on other types of cathodes conventionally employed in acid nickel plating processes utilizing solutions of the type indicated herein.

Table III

|                                                                                                                               | Grams per Liter |       |       |       |
|-------------------------------------------------------------------------------------------------------------------------------|-----------------|-------|-------|-------|
| NiSO <sub>4</sub> ·7H <sub>2</sub> O                                                                                          | 300             | 300   | 300   | 300   |
| NaCl <sub>2</sub> ·6H <sub>2</sub> O                                                                                          | 40              | 40    | 40    | 40    |
| H <sub>3</sub> BO <sub>3</sub>                                                                                                | 40              | 40    | 40    | 40    |
| Sodium lauryl sulfate                                                                                                         | 0.15            | 0.15  | 0.15  | 0.15  |
| 1,2-ethylene-bis(B-cyanoethyl-ethylsulfonium ethylsulfate)                                                                    | 0.15            | ----- | ----- | ----- |
| methyl-bis(B-cyanoethyl) sulfonium p-tolueno sulfonate                                                                        | 0.01            | ----- | ----- | ----- |
| B-cyanoethyl propylethylsulfonium ethyl sulfate                                                                               | -----           | 0.01  | ----- | ----- |
| Ethyl bis(B-cyanoethyl) sulfonium ethyl sulfate                                                                               | -----           | ----- | 0.01  | ----- |
| [C <sub>6</sub> H <sub>5</sub> SC <sub>2</sub> NHSC <sub>2</sub> NH <sub>2</sub> C <sub>6</sub> H <sub>5</sub> ] <sub>2</sub> | 3               | 3     | 3     | 3     |
| [C <sub>6</sub> H <sub>5</sub> SC <sub>2</sub> NHSC <sub>2</sub> NH <sub>2</sub> O] <sub>2</sub>                              | 40              | 40    | 40    | 40    |
| Current Density a.s.f.                                                                                                        | 140             | 140   | 140   | 140   |
| Temperature range °F                                                                                                          | 75              | 75    | 75    | 75    |

What I claim is:

1. An aqueous acid nickel plating solution comprising a source of nickel ions selected from the class consisting of nickel sulfate, nickel chloride and mixtures thereof, said solution also containing cooperating additives for enhancing the brightness of nickel deposits produced therein, one of said additives being present in a concentration of from 0.05 to 20 grams per liter and being chosen from the class consisting of aromatic sulfonates, aromatic sulfonamides, aromatic sulfimides, aliphatic sulfonamides and sulfonic acids, and the second being present in a concentration of from 0.0025 to 0.075 gram per liter and being chosen from the class of compounds having the formula



wherein R is a member selected from the group consisting of —H, —CN,



W is a hydrocarbon radical; X is an acid radical selected from the group consisting of sulfate, sulfonate, halide and perchlorate radicals; n is an integer from 1 to 6 and n' is an integer from 1 to 6.

2. An aqueous, acid, nickel plating solution comprising nickel plating solution comprising nickel sulfate and nickel chloride and cooperating additives being present in a concentration from 0.05 to 20 grams per liter and, one of said additives being chosen from the class consisting of aromatic sulfonates, aromatic sulfonamides, aromatic sulfimides, aliphatic sulfonamides and sulfonic acids and the other of said cooperating additives being a compound of the formula



and being dissolved in said solution in concentration from 0.0025 to 0.075 gram per liter.

3. An aqueous, acid, nickel plating solution comprising nickel plating solution comprising nickel sulfate and nickel chloride and cooperating additives, one of said additives being present in the concentration of from 0.05 to 20 grams per liter and being chosen from the class consisting of aromatic sulfonates, aromatic sulfonamides, aromatic sulfimides, aliphatic sulfonamides and sulfonic acids and 10 the other of said cooperating additives being a compound of the formula



15 and being dissolved in said solution in concentration from 0.0025 to 0.075 gram per liter.

4. An aqueous, acid, nickel plating solution comprising nickel plating solution comprising nickel sulfate and nickel chloride and cooperating additives, one of said additives 20 being present in a concentration of from 0.05 to 20 grams per liter and being chosen from the class consisting of aromatic sulfonates, aromatic sulfonamides, aromatic sulfimides, aliphatic sulfonamides and sulfonic acids and the other of said cooperating additives being a compound of the formula



and being dissolved in said solution in concentration from 0.0025 to 0.075 gram per liter.

- 30 5. An aqueous, acid, nickel plating solution comprising nickel plating solution comprising nickel sulfate and nickel chloride and cooperating additives, one of said additives being present in a concentration of from 0.05 to 20 grams per liter and being chosen from the class consisting of aromatic sulfonates, aromatic sulfonamides, aromatic sulfimides, aliphatic sulfonamides and sulfonic acids and the other of said cooperating additives being a compound of the formula



and being dissolved in said solution in concentration from 0.0025 to 0.075 gram per liter.

- 45 6. An aqueous, acid, nickel plating solution comprising nickel plating solution comprising nickel sulfate and nickel chloride and cooperating additives, one of said additives being present in a concentration of from 0.05 to 20 grams per liter and being chosen from the class consisting of aromatic sulfonates, aromatic sulfonamides, aromatic sulfimides, aliphatic sulfonamides and sulfonic acids and the other of said cooperating additives being a compound of the formula



55 and being dissolved in said solution in concentration from 0.0025 to 0.075 gram per liter.

- 60 7. An aqueous, acid, nickel plating solution comprising nickel plating solution comprising nickel sulfate and nickel chloride and cooperating additives, one of said additives being present in a concentration of from 0.05 to 20 grams per liter and being chosen from the class consisting of aromatic sulfonates, aromatic sulfonamides, aromatic sulfimides, aliphatic sulfonamides and sulfonic acids and the other of said cooperating additives being a compound of the formula



65 and being dissolved in said solution in concentration from 0.0025 to 0.075 gram per liter.

No references cited.

UNITED STATES PATENT OFFICE  
CERTIFICATION OF CORRECTION

Patent No. 2,972,571

February 21, 1961

Jack L. Towle

It is hereby certified that error appears in the above numbered patent requiring correction and that the said Letters Patent should read as corrected below.

Column 2, line 13, for "theg roup" read -- the group --; Column 2, line 23, for "XX" read -- X --; line 34, strike out "radical"; columns 1 and 2, Table 1, second column, under the heading "Structure", and opposite item No. 6, the formula should appear as shown below instead of as in the patent:



column 5, line 64 to column 6, line 2, claim 2 should appear as shown below instead of as in the patent:

2. An aqueous, acid, nickel plating solution comprising nickel plating solution comprising nickel sulfate and nickel chloride and cooperating additives, one of said additives being present in a concentration from 0.05 to 20 grams per liter and being chosen from the class consisting of aromatic sulfonates, aromatic sulfonamides, aromatic sulfimides, aliphatic sulfonamides and sulfonic acids and the other of said cooperating additives being a compound of the formula  $NC-CH_2-CH_2-S-CH_2-CH_2-CN$ , and being



5215 2 2 3

dissolved in said solution in concentration from 0.0025 to 0.075 gram per liter.

Signed and sealed this 18th day of July 1961.

(SEAL)

Attest:

ERNEST W. SWIDER

**Attesting Officer**

**DAVID L. LADD**  
Commissioner of Patents